

# United States Patent [19]

Takashima

[11] 3,883,347

[45] May 13, 1975

[54] **SLAG-FORMING AGENT FOR STEELMAKING**

[75] Inventor: **Masaru Takashima, Tokyo, Japan**

[73] Assignee: **Aikoh Co. Ltd., Tokyo, Japan**

[22] Filed: **Sept. 27, 1973**

[21] Appl. No.: **401,269**

## Related U.S. Application Data

[63] Continuation-in-part of Ser. No. 225,286, Feb. 10, 1972, abandoned.

## Foreign Application Priority Data

Feb. 16, 1971 Japan ..... 46-6491

[52] U.S. Cl. ..... **75/30; 75/58; 75/93 A; 75/94; 75/96; 164/56**

[51] Int. Cl. ..... **C21c 5/54**

[58] Field of Search ..... 75/30, 93 A, 96, 53-58, 75/93 G, 94; 148/26, 24; 164/56, 57

## References Cited

### UNITED STATES PATENTS

1,002,133 8/1911 Bryant et al. ..... 75/93 A

|           |         |                     |          |
|-----------|---------|---------------------|----------|
| 1,331,816 | 2/1920  | McKnight, Jr. ....  | 164/56   |
| 2,748,040 | 5/1956  | Conn .....          | 148/26   |
| 3,214,806 | 11/1965 | Fox et al. ....     | 75/96 X  |
| 3,234,608 | 2/1966  | Peras .....         | 164/56 X |
| 3,414,042 | 12/1968 | Behrens et al. .... | 164/57   |
| 3,731,868 | 5/1973  | Arikawa et al. .... | 75/94 X  |

## FOREIGN PATENTS OR APPLICATIONS

570,480 2/1959 Canada ..... 164/57

Primary Examiner—Allen B. Curtis

Assistant Examiner—Thomas A. Waltz

Attorney, Agent, or Firm—D. Paul Weaver

[57]

## ABSTRACT

A method of making steel comprising adding to molten steel a slag-forming agent comprising from 2 to 20% by weight of metallic titanium particles having a size of 0.5 to 20 mm., 30 to 94% by weight of aluminum oxide, and a binder.

7 Claims, No Drawings

## SLAG-FORMING AGENT FOR STEELMAKING

## BACKGROUND OF THE INVENTION

This application is a continuation-in-part of Ser. No. 225,286, filed Feb. 10, 1972, now abandoned.

The present invention relates to a method of making steel using a slag-forming agent which is added to the steel in the furnace.

Limestone, fluorspar, scrap of silica brick, or a mixture thereof have been conventionally used as a slag-forming agent in making steel in a converter, an electric furnace, or an open hearth furnace. Fluorspar has been the preferred slag-forming agent in steelmaking because it improves the fluidity of the slag and is economical. However, fluorspar ( $\text{CaF}_2$ ) is a fluoride, and generates fluorine gas during the steelmaking process which damages the walls of the furnace and obstructs the working environment. Although fluorspar ideally should contain more than 85% by weight of  $\text{CaF}_2$  when used in steelmaking, many available fluorspars are short in  $\text{CaF}_2$  content and so are not as desirable for use in steelmaking.

It has been discovered that aluminum ash consisting of mainly aluminum oxide and containing metallic aluminum deoxidizes the slag in steelmaking. For example, the aluminum ash reduces chromium oxide in the slag of chromium alloy steel to metallic chromium, thereby adding more chromium to the molten steel to increase the amount of chromium in the molten steel. This in turn reduces the amount of fluorspar needed, and accelerates the speed of slag-formation and shortens the reducing time.

However, the metallic aluminum ash in the molten steel, even if it is a fine powder, remains in the molten steel as aluminum oxide, which has a deleterious effect on the molten steel. At the same time, when it is used in continuous casting of molten steel, the aluminum oxide present in the molten steel adheres to and clogs the nozzle of the tundish, and makes casting impossible by combining with manganese oxide or silicon dioxide. Additionally, aluminum is very reactive with oxygen and is instantaneously oxidized at the high temperature inside the furnace so that the amount of aluminum available as a deoxidizing agent is only 30-50% of that added to the melt. This makes aluminum very expensive as a slag-forming agent, as well as very inefficient.

## SUMMARY OF THE INVENTION

The object of the present invention is to provide a process for making steel which does not have the disadvantages of methods using the above-described slag-forming agents.

According to the present invention, steel is made by incorporating into the molten steel a slag-forming agent containing metallic titanium as well as aluminum oxide. This slag-forming agent deoxidizes molten steel, and the resulting titanium oxide floats easily on the molten steel so that it can be readily removed therefrom. Therefore, even in the continuous casting of molten steel, the titanium dioxide does not clog the nozzle of the tundish. As metallic titanium does not react with oxygen as readily as aluminum does, it is not oxidized instantaneously, and almost all of the metallic titanium is available as an oxidizing agent for a long time. The method of the present invention accelerates the speed of slag-forming, reduces the amount of fluorspar used,

and results in an improved dephosphorizing and desulfurizing rate as compared with prior art methods.

The slag-forming agent for use in the method according to the present invention comprises from 2 to 20% by weight of metallic titanium particles having a size of 0.5 to 20 mm., 30 to 94% by weight of aluminum oxide, and 4 to 20% by weight of a binder.

As metallic titanium or titanium alloy containing in excess of 80% by weight of titanium metal is expensive, 10 it is most economical to use scraps. Less than 2% by weight of titanium in the slag-forming agent is ineffective, and more than 20% by weight to titanium does not give a greater effect than 20%. The size of the metallic titanium particles is limited to 0.5 mm. to 20 mm. to enhance the speed of the reaction. The titanium is more easily oxidized and thus is less effective at particle sizes below 0.5 mm., and the reaction is too slow when the particle size exceeds 20 mm.

Although alumina brick powder, bauxite, aluminum 20 ash or aluminum dross are a preferable material for supplying aluminum oxide in the slag-forming agent of the present invention, other alumina containing materials can be also used. The aluminum ash is a slag which is formed when metallic aluminum is refined and the aluminum dross is a floating slag which is formed when metallic aluminum is remelted. Although the aluminum ash or dross has a defect in that its composition is not uniform, these materials, which contain as a main component aluminum oxide and also contain some metallic aluminum, are formed from the slag which is developed when metallic aluminum is refined or remelted and oxides are formed from the flux. Therefore, these materials are economically beneficial and preferable.

Also, it is desirable to use various kinds of synthetic 35 resin binders, organic binders such as animal or vegetable glue, starch and dextrin, or inorganic binders such as various kinds of cement, water glass and bentonite to make the slag-forming agent according to the present invention, into a molding of a 10-50 mm. briquette, tablet or pellet by a roll pressing machine or a granulating tablet-making machine. The organic binder is preferably used in a quantity of 4 to 12% by weight and the inorganic binder is preferably used in a quantity of 7 to 40 20% by weight.

## DESCRIPTION OF THE PREFERRED EMBODIMENTS

The present invention is illustrated by the following 50 examples.

Examples using the slag-forming agent according to the present invention are shown in Table 1 in comparison with the prior slag-forming agent.

TABLE 1

| Material                                                | Composition and Shape of Slag-Forming Agent (% by weight) |    |   |   | Conventional Slag Forming Agent |  |
|---------------------------------------------------------|-----------------------------------------------------------|----|---|---|---------------------------------|--|
|                                                         | Slag-Forming Agent of the Present Invention               |    |   | D |                                 |  |
|                                                         | A                                                         | B  | C |   |                                 |  |
| <u>Alumina Line Materials</u>                           |                                                           |    |   |   |                                 |  |
| Aluminum ash<br>( $\text{Al}_2\text{O}_3$ content: 65%) | 75                                                        | 50 | — | — | —                               |  |
| (Metallic aluminum: 15%)                                | —                                                         | —  | — | — | 92                              |  |
| Aluminum ash<br>( $\text{Al}_2\text{O}_3$ content: 60%) | —                                                         | —  | — | — | —                               |  |
| (Metallic aluminum: 24%)                                | —                                                         | —  | — | — | —                               |  |

3  
TABLE 1-Continued

| Material                                                                  | Composition and Shape of Slag-Forming Agent (% by weight) |    |    |                                 |
|---------------------------------------------------------------------------|-----------------------------------------------------------|----|----|---------------------------------|
|                                                                           | Slag-Forming Agent of the Present Invention               |    |    | Conventional Slag Forming Agent |
|                                                                           | A                                                         | B  | C  | D                               |
| Bauxite<br>(Al <sub>2</sub> O <sub>3</sub> content: 57%)                  | —                                                         | 27 | 72 | —                               |
| Titanium and Its Alloys                                                   |                                                           |    |    |                                 |
| Titanium metal<br>(Size: 2-6 mm.)<br>(Purity: 99.3%)                      | 10                                                        | —  | 20 | —                               |
| Titanium alloy<br>(Size: 5-20 mm.)<br>(Titanium content: 87%)             | —                                                         | 15 | —  | —                               |
| Binder                                                                    |                                                           |    |    |                                 |
| Self-hardening phenol resin<br>(Solid component of 60% methanol solution) | —                                                         | 8  | 8  | 8                               |
| Portland cement                                                           | 15                                                        | —  | —  | —                               |
| Size of Molding (mm.)<br>(Briquette)                                      | 25                                                        | 25 | 25 | 25                              |

## Test 1

Heat resistant steel containing chromium (formed of 0.4-0.5% carbon, 3-3.5% silicon, less than 0.6% manganese, 7.5-9.5% chromium, less than 0.03% phosphorus, less than 0.003% sulfur, and iron as the remainder) was melted in a 5 ton electric furnace and the slag-forming agent (A, B, and C) according to the present invention, having the said composition and size (Table 1) and the conventional slag-forming agent (D), were added respectively as shown in Table 2, and the steel, after being made, was cast by a continuous casting method.

could not be done. However, in the case of Nos. 1, 2 and 3, when the slag-forming agents (A, B, and C), containing metallic titanium according to the present invention, were used, smooth casting was possible without clogging the nozzle. Also, by adding smaller amount of the slag-forming agents (A, B and C) according to the present invention compared to the conventional slag-forming agent, the yield of chromium added, as shown in Table 2, was improved and the reduction time could be shortened because of the rapid rate in which the slag was formed.

## Test 2

Each of the slag-forming agents (A, B and C) according to the present invention and the conventional slag-forming agent (D) having the same composition and size (Table 1) and fluorspar were charged together with scrap at the time of making common steel by a 100 ton converter operation, and blowing was done by an ordinary operation. The results are shown in Table 3. Nos. 1 and 2 are the results when only fluorspar was used. Nos. 3 and 4 are the results when the conventional slag-forming agent (D) was used, and Nos. 5 through 10 are the results when the slag-forming agents (A, B and C) relating to the present invention were used.

As shown in Table 3, by using about 1 kilogram per ton of the slag-forming agents (A, B and C) according to the present invention, the amount of fluorspar used could be decreased by approximately 3 kilograms per ton compared to the time when only fluorspar (Nos. 1 and 2) was used, and the amount of fluorspar used could be slightly decreased compared to the time when conventional slag-forming agent (D) (Nos. 3 and 4) was used. Further, the deposphorizing rate and the desulfurizing rate could be improved and the steelmaking time could be shortened because of the rapid rate at

TABLE 3

|                                                                         | Comparative Table on the Results of Using Slag-Forming Agent |      |      |      |      |      |      |      |      |      |
|-------------------------------------------------------------------------|--------------------------------------------------------------|------|------|------|------|------|------|------|------|------|
|                                                                         | 1                                                            | 2    | 3    | 4    | 5    | 6    | 7    | 8    | 9    | 10   |
| Amount used of limestone (kg/t)                                         | 60.4                                                         | 60.5 | 60.2 | 60.5 | 60.3 | 59.8 | 60.3 | 60.5 | 60.2 | 60.5 |
| Amount of fluorspar (kg/t)                                              |                                                              |      |      |      |      |      |      |      |      |      |
| Charging in advance                                                     | 3.0                                                          | 3.0  | 2.0  | 2.0  | 2.0  | 2.0  | 2.0  | 2.0  | 2.0  | 2.0  |
| Charging later                                                          | 2.4                                                          | 2.5  | 1.0  | 0.8  | 0.4  | 0.3  | 0.2  | 0.2  | 0.2  | 0.2  |
| Amount of slag-forming agent according to the present invention (kg/t)* | A                                                            | —    | —    | —    | 1.0  | 1.0  | —    | —    | —    | —    |
| B                                                                       | —                                                            | —    | —    | —    | —    | —    | 1.0  | 1.0  | —    | —    |
| C                                                                       | —                                                            | —    | —    | —    | —    | —    | —    | —    | 1.0  | 1.0  |
| D                                                                       | —                                                            | —    | —    | 1.2  | 1.3  | —    | —    | —    | —    | —    |
| Amount of conventional slag-forming agent (kg/t)*                       |                                                              |      |      |      |      |      |      |      |      |      |
| Deposphorizing rate (%)                                                 | 89.3                                                         | 88.6 | 89.5 | 90.4 | 90.8 | 90.5 | 92.3 | 91.8 | 91.3 | 90.8 |
| Desulfurizing rate (%)                                                  | 35.2                                                         | 35.4 | 34.6 | 36.3 | 38.1 | 38.8 | 40.1 | 39.5 | 38.6 | 39.1 |

\*Charging in advance.

TABLE 2

| Slag-Forming Agent Added | Comparative Table on the Results of Using Slag-Forming Agent |       |       |       |
|--------------------------|--------------------------------------------------------------|-------|-------|-------|
|                          | No.1                                                         | No.2  | No.3  | No.4  |
| A (kg)                   | 200                                                          | —     | —     | —     |
| B (kg)                   | —                                                            | 190   | —     | —     |
| C (kg)                   | —                                                            | —     | 185   | —     |
| D (kg)                   | —                                                            | —     | —     | 230   |
| Yield of Chromium Added  | 98.3%                                                        | 97.8% | 98.9% | 91.6% |

In the case of No. 4, when the conventional slag-forming agent (D) was used, the nozzle of the tundish was clogged during continuous casting and casting

which the slag-forming agent according to the present invention forms the slag. Therefore, the slag-forming agent according to the present invention was found to be desirable.

As described above, by making steel using a slag-forming agent containing metallic titanium, there is no danger of titanium dioxide remaining in the molten steel. In the case of continuous casting, there is no clogging of the nozzle of the tundish and deoxidation of the slag. For example, the chromium content of steel made according to the present invention is higher than the chromium content of steel made according to the prior art process. Additionally, the steelmaking time per charge is reduced because of the rapid rate at which slag is formed as compared with the prior art process. Thus, efficiency of the steelmaking process is

improved. Further, the amount of fluorspar necessary can be decreased and the desulfurization and dephosphorization rates can be improved.

What is claimed is:

1. A method for making steel comprising adding to molten steel a slag-forming agent comprising 2 to 20% by weight of metallic titanium particles, 30 to 94% by weight of aluminum oxide, and 4 to 20% by weight of a binder.

2. The method of claim 1 wherein the metallic titanium particles range from 0.5 mm. to 20 mm.

3. The method of claim 1 wherein the metallic titanium particles are in the form of titanium alloy containing at least 80% by weight of metallic titanium.

4. The method of claim 1 wherein the aluminum oxide is selected from the group consisting of alumina brick powder, bauxite powder, aluminum ash, and aluminum dross.

5. The method of claim 1 wherein the binder is selected from the group consisting of synthetic resin, animal glue, vegetable glue, starch and dextrin.

6. The method of claim 1 wherein the binder is selected from the group consisting of cement, water glass, and bentonite.

7. The method of claim 1 wherein the slag-forming agent is in the form of a molding selected from the group consisting of a briquette, a tablet, and a pellet.

\* \* \* \* \*